

## UNITED STATES PATENT OFFICE

STANLEY D. SHIPLEY, OF STAMFORD, CONNECTICUT, ASSIGNOR TO ATLAS POWDER COMPANY, OF WILMINGTON, DELAWARE, A CORPORATION OF DELAWARE

## BRUSHING LACQUER

No Drawing.

Application filed October 21, 1925. Serial No. 64,029.

This invention relates to nitrocellulose lacquers and lacquer enamels and it has for its object to provide an improved substance of this character of such composition that it can be successfully applied over previously applied coats of paint, varnish or nitrocellulose lacquer or lacquer enamel, without attacking such previously applied coats.

Where an attempt has been made to apply a lacquer or lacquer enamel, consisting of a nitrocellulose base, and the commonly known solvents, upon old work, that is, upon surfaces which have been previously coated with paint, varnish or nitrocellulose lacquer or lacquer enamel, the solvent content of the newly applied coat has attacked and softened the undercoating and it has not been possible to get a good finish. This is particularly true if the application of the newly applied coat is with a brush, where the mechanical action of the brush tends to dislodge and slough off the softened undercoatings.

One of the reasons why it has not been possible to successfully apply these nitrocellulose lacquers and lacquer enamels with a brush, even upon new surfaces, is that the solvents commonly employed, dry or evaporate with such rapidity that "pulling" develops before the brushing can be completed, with the result that a smooth surface cannot be secured.

To avoid the foregoing difficulties and to produce a nitrocellulose lacquer or lacquer enamel which may be successfully applied in any suitable way, including brushing, and either upon new work or over previously applied coatings, I reduce the amount of active solvent in the lacquer to a quantity just sufficient to keep the nitrocellulose in solution and I employ, in conjunction therewith, a substantial proportion of a diluent consisting of a petroleum hydrocarbon, such as gasoline.

As hereinafter set forth, I employ as much as 37½% of gasoline, and this large proportion of gasoline so attenuates or dilutes the solvent of the lacquer that the latter will not appreciably attack previously applied undercoatings of the class described, namely, paints, varnishes, nitrocellulose lacquers, or lacquer enamels. Paints, as commonly

known, contain oils and nitrocellulose, paints, lacquers or enamels practically always contain resins or gums. Gasoline is either a poor solvent or a non-solvent for these substances and, consequently, will not itself appreciably attack undercoatings of the character described, and at the same time, when used in the large proportions stated, it prevents the solvent of the present lacquer from attacking such previously applied undercoats. I do not claim to be the first to use gasoline as a diluent in nitrocellulose lacquers, nor to be the first to have discovered that gasoline may be used as a diluent in nitrocellulose lacquers, but so far as I am aware, what is new with me is the conception of the thought of using in a brushing lacquer, a very large proportion of a diluent having, upon the one hand, the characteristic that, despite the large proportion of the same present, it exercises no appreciable softening effect upon the previously applied coats of paint, lacquer, varnishes, and the like, and, in addition, when used in such large proportions, so dilutes the solvent content of the lacquer as to prevent that element of the composition from attacking such undercoats.

In the specific proportions hereinafter recited, I disclose the use of other diluents in conjunction with the gasoline, in the present instance, specifically, toluol. In the absence of the gasoline, toluol would attack previously applied coatings of paint, varnish, lacquer, and the like, but when gasoline, in the proportions recited is used, the resultant dilution of the toluol is so great that it does not then appreciably attack such undercoatings. Further, it will be recognized by any one skilled in the art, that the nitrocellulose solvents employed in my composition would attack undercoatings of the character recited, if not associated with the considerable proportion of harmless diluent set forth in the example recited, (gasoline).

In my copending application, Serial No. 59,164 filed on the 28th day of September, 1925, I have claimed a lacquer analogous to that claimed herein. However, in the application aforesaid, the claims are devoted to the protection of the thought of utilizing,

in a lacquer of the character described, a slow drying solvent, (specifically ethyl glycol). The present application is intended to cover the broad thought of reducing the amount of active solvent in the lacquer to a quantity just sufficient to keep the nitrocellulose in solution and the employment of a diluent, of such a nature that the diluent will not, itself, exercise any undesirable effect upon undercoatings. The present application is intended to cover the thought outlined above, irrespective of whether such solvent is materially slower drying than the solvents commonly employed in nitrocellulose solutions, or not.

15 The following composition will yield a lacquer which will not undesirably effect undercoatings.

|                | Per cent |
|----------------|----------|
| Ethyl acetate  | 8        |
| 20 Camphor oil | 1.5      |
| Butyl acetate  | 20.5     |
| Gasoline       | 27.5     |
| Toluol         | 37.5     |
| Resin solution | 5        |
|                | 100      |

25 Nitrocellulose 3 oz. per gallon  
In addition to the resin solution above mentioned, I contemplate incorporating pigments (zinc oxide for example) to make lacquer enamels.

It should be understood that the above recited formula is merely illustrative. It is not necessary that the diluents used consist wholly of gasoline or other petroleum hydrocarbon. Other diluents may be present. It is only necessary that a substantial proportion of the diluent be of a nature, such that it will have no destructive effect upon 35 previously applied coatings. Most of the commonly used diluents, such as toluene or benzene, for example, are, themselves, destructive of undercoatings when used in a lacquer. Furthermore, it is of importance 40 that the rates of evaporation of the solvent and the diluent employed be such as to insure the evaporation of the diluent ahead of the complete evaporation of the solvent, since otherwise the nitrocellulose would be precipitated from the solution and the nitrocellulose film would be spoiled. It would be 45 hazy, very weak and probably non-adherent.

When making nitrocellulose lacquers containing resins, the gum solution is added to 55 the nitrocellulose solution. It is sometimes desirable to employ small quantities of toluol or alcohol as solvents for the resin in making the gum solution. However the quantity of resin solvent required is so small as to exert 60 no appreciable deleterious effect on previously applied undercoatings and it is to be understood that substances used primarily as resin solvents are not to be considered diluents within the meaning of the appended 65 claim.

I am aware of the fact that it is common practice to use gasoline as a diluent in nitrocellulose solvent compositions. However, to the best of my knowledge and belief, gasoline has never been designedly employed in the 70 particular proportions and for the purposes, outlined herein, nor am I aware that it has ever been employed in such proportions and with a solvent of such a nature, as to insure the evaporation of the diluent ahead of the 75 evaporation of the solvent, to the end of producing a lacquer which can be applied by spraying, dipping or brushing and yet give a smooth finish, and which will not attack undercoats, either through the action of the 80 solvent or the action of the diluent.

Having described my invention, what I claim is:

A lacquer composition comprising the following ingredients, combined in substantially the proportions stated, viz:

|                | Per cent |
|----------------|----------|
| Ethyl acetate  | 8        |
| Camphor oil    | 1.5      |
| Butyl acetate  | 20.5     |
| Gasoline       | 37.5     |
| Toluol         | 27.5     |
| Resin solution | 5        |
|                | 100      |

combined with nitrocellulose 3 ozs. per gallon.

In testimony whereof he affixes his signature.

STANLEY D. SHIPLEY.

100

105

110

115

120

125

130